

## UNITED STATES PATENT OFFICE

2,032,554

AUTO-OXIDATION AND POLYMERIZATION  
CATALYSTFranciscus Visser't Hooft, Buffalo, N. Y., assignor  
to Lucidol Corporation, Buffalo, N. Y., a corpora-  
tion of DelawareNo Drawing. Application August 3, 1933,  
Serial No. 683,544

## 5 Claims. (Cl. 134—56)

The present invention relates to a new auto-oxidation and polymerization catalyst and to methods of employing the same in various processes including the drying of those drying oils which contain elaeostearin. More particularly the present invention relates to organic peroxides properly so-called, and their use in such drying oils as China-wood oil and similar oils, which consist largely of elaeostearin. As is well known, tung oil (or China-wood oil) of average quality contains about 85% of elaeostearin.

The drying of so-called drying oils is a complicated process in which polymerizations are accompanied, preceded or followed by oxidations. According to Eibner (Das Oelrocknen, 1930), drying of oils is due to auto-oxidation and polymerization. In the case of raw linseed oil, Eibner states that drying is due to auto-oxidation, in raw China-wood oil to auto-oxidation and polymerization. In "bodied" oils, that is oils of which the viscosity has been increased, a certain polymerization occurs during the bodying process. The drying process of "bodied" oils involves the formation of films from partly polymerized products under the influence of auto-oxidation.

It was old prior to the present invention to use (with all types of drying oils) oil drying agents such as metal oxides, metal soaps, metal resinates, and the like to accelerate the drying under atmospheric conditions. The use of these driers has various disadvantages in that they unfavorably affect the stability of the oil films produced by the drying of the oil, causing a tendency to wrinkle, also checking and cracking of the films, decreasing the water resistance of the films, decreasing the life of the films and other highly undesirable effects. The reason for most of these unfavorable effects caused by the driers is the fact that they catalyze for the most part, the auto-oxidation of the drying oils, without appreciably accelerating the polymerization.

It was also known prior to the present invention that organic peroxides have a bleaching action on oils (not readily drying oils), see U. S. Patents 901,718; 1,854,764; 1,687,804.

It was also old prior to the present invention to use substances such as "rubrene peroxide" to accelerate drying of the oil contained in a printing ink by heating the ink containing the "rubrene peroxide" distributed throughout the mass thereof (see U. S. Patent 1,842,196). However the term "rubrene peroxide" is now generally considered to be a misnomer and the most recent investigations indicate that it is an oxide capable of dissociation into rubrene and oxygen, and not possessing the

characteristic properties of a true peroxide. These comments are pertinent as will appear more fully hereinafter, because I employ a true organic diacyl peroxide, such as dibenzoyl peroxide, in effecting an acceleration of the drying of an oil of the China-wood oil type. These diacyl peroxides, as distinguished from rubrene peroxide, are not capable of dissociation to liberate free oxygen by heating.

I have now found that drying oils of the type of China-wood oil, i. e., oils containing elaeostearin, can be dried under atmospheric conditions without the use of any of the above mentioned or any other commercial driers, by the addition of diacyl peroxides to the oils. These diacyl peroxides are catalysts which accelerate the natural rate of drying of the oils. They do not considerably accelerate the drying of oils of the type of linseed oil. The mechanism of the drying operation of oils of the type of linseed oil involves auto-oxidation. Only in the case of drying oils of the type of China-wood oil where both auto-oxidation and polymerization are involved, the diacyl peroxides accelerate the rate of drying, to any commercially useful extent.

While dibenzoyl peroxide and other organic peroxides have been used heretofore to bleach oils, no one prior to the present invention realized the potentiality of these peroxides as specific drying accelerators for oils of the type of China-wood oil.

A further advantage of the diacyl peroxides is that they are completely soluble in the oils in the amounts used and do not precipitate from the oils as do the ordinary commercial driers.

The following examples will further illustrate the application of the principle of my invention.

## Example I.

A quick drying paint is produced by mixing the following materials and grinding them in a paint mill, for example a pebble mill:

|                             | Pounds | 45 |
|-----------------------------|--------|----|
| Zinc oxide                  | 250    | 45 |
| Bodied China-wood oil       | 250    |    |
| Mineral spirits             | 70     |    |
| Powdered dibenzoyl peroxide | 2.3    |    |

This paint, when brushed onto a board, will dry in the air in 4-5 hours, when poured on glass in 7-8 hours, while a similar paint made with the same ingredients but without dibenzoyl peroxide  $(C_6H_5CO)_2O_2$  will still be wet on the board in 6 hours and on the glass even after 48 hours.

## Example II

A quick drying printing ink can be prepared by grinding 75 pounds of carbon black and 3 pounds of indigo with 100 pounds of tung oil in a levigating mill and then adding to this base a mixture of 5½ pounds of dilauroyl peroxide  $(C_{11}H_{20}CO)_2O_2$  and 5½ pounds of rosin oil. This ink will dry completely in the so-called "hot plate test" at 100° C. in less than 8 seconds. 5  
 10 This hot plate test consists in smearing some of the ink upon a glass plate which is maintained at 100° C., and noting the time when the ink has dried sufficiently so that it will not smear when touched by the operator with a clean finger. 15  
 15 These diacyl peroxides can be used as ingredients in regular stock inks containing China-wood oil but their action on the elaeostearin is so pronounced that under ordinary storage conditions, even after a short time, "skinning" and 20  
 20 "livering" of the inks caused by premature oxidation and polymerization, occurs. Certain inhibitors may counteract this effect of the diacyl peroxides, but usually the inhibitors react chemically with the diacyl peroxides, thereby slowly 25  
 25 converting the peroxides into non-accelerators and the useful effect of the peroxides is thereby lost.

The particular ink of Example II, containing 30 no inhibitor, must be used immediately, and cannot be left even for a few days without livering.

## Example III

A quick drying raw China-wood oil is prepared by adding 6 ounces of dimyristoyl peroxide  $(C_{13}H_{22}CO)_2O_2$  to 100 pounds of raw China-wood oil and stirring the oil at room temperature until all the peroxide is dissolved. 35

While an untreated oil gave a drying test of 18 hours, the treated oil dried under the same conditions in 4 hours. 40

## Example IV

A quick drying bodied China-wood oil is produced by adding 3½ ounces of mm' ditolyl peroxide  $(CH_3C_6H_4CO)_2O_2$  to 100 pounds of bodied China-wood oil and stirring the oil at 40-60° C. until the peroxide has dissolved. Such a treated oil will dry in 4 hours against a drying time of 18-24 hours for the untreated bodied oil. 45

## Example V

An example of a rapid drying varnish containing a diacyl peroxide is prepared as follows: To 50 100 pounds of any varnish gum and 250 pounds of tung oil properly cooked and thinned with 100 pounds of mineral spirits, and 1 pound of pp' ditolyl peroxide  $(CH_3C_6H_4CO)_2O_2$ . The above varnish dried hard in seven hours, while the 55 same varnish omitting pp' ditolyl peroxide required 23 hours to dry under the same conditions.

The diacyl peroxides disclosed in the above examples are true organic peroxides or derivatives of hydrogen peroxide and possess the characteristic oxygen bridge  $O-O$ . Diacyl peroxides are derived from  $H_2O_2$  by replacement of the two hydrogen atoms by one or two acyl groups. The best known diacyl peroxide is dibenzoyl peroxide  $(C_6H_5CO)_2O_2$ . These diacyl peroxides differ from "rubrene peroxide" in that they do not liberate free oxygen when heated and are not subject to a dissociation or reversible oxidation. 65

But one of the oxygen atoms of the diacyl peroxide molecule is "active" i. e. seems to function 70

as a powerful catalyst, and is quite different chemically and acts differently from the "free oxygen" which is liberated from substances such as rubrene peroxide. For the purpose of clarity and simplification of the explanation of the invention, the per cent of diacyl peroxide used with the oil to polymerize the same and also the per cent of "active oxygen" with reference to the said oils are tabulated below, the second table being based on the specific examples, each item identifying the particular example on which it is based. 10

## Active oxygen content of diacyl peroxides

|                      |       |    |
|----------------------|-------|----|
| Dibenzoyl peroxide   | 6.61% | 15 |
| Dilauroyl peroxide   | 4.02% |    |
| Dimyristoyl peroxide | 3.52% |    |
| pp' ditolyl peroxide | 5.92% |    |
| mm' ditolyl peroxide | 5.92% |    |

The following table also gives the amount of diacyl peroxide in percentage of oil as used in the five examples given in the patent application. In this same table we also calculated the active oxygen in percentages of oil: 20

|                                                                   | Diacyl peroxide percentage, based on oil | Active oxygen percentage, based on oil |
|-------------------------------------------------------------------|------------------------------------------|----------------------------------------|
| Example 1—<br>250 pounds oil<br>2.3 pounds benzoyl peroxide       | Per cent<br>0.92                         | Per cent<br>0.0610                     |
| Example 2—<br>100 pounds oil<br>5.5 pounds dilauroyl peroxide     | 5.5                                      | 0.2211                                 |
| Example 3—<br>100 pounds oil<br>6 ounces dimyristoyl peroxide     | 0.375                                    | 0.0132                                 |
| Example 4—<br>100 pounds oil<br>3½ ounces mm' ditolyl peroxide    | 0.219                                    | 0.0130                                 |
| Example 5—<br>250 pounds tung oil<br>1 pound pp' ditolyl peroxide | 0.4                                      | 0.0237                                 |

The diacyl peroxides act in a wholly unexpected manner as catalysts for the polymerization or auto-oxidation under atmospheric conditions of oils of the type of China-wood oil, containing elaeostearin. Its apparent action is on compounds with the triple conjugated system: 45



This action is accelerated further by heat, light or oxygen or by a combination of these. At ordinary room temperature and in diffused daylight there is a distinct accelerating action produced however by the diacyl peroxides which causes faster drying of the oil. 50

The application of the principle of my invention is not limited to the above examples. Other applications of the catalytic action of diacyl peroxides on oils of the type of China-wood oil will be obvious, such as impregnating pulp, paper and woven fabrics, etc. For example, an oil-proof container made by impregnating a container constructed from paper, wood pulp or cardboard with tung oil and a small amount of a diacyl peroxide and hardening the tung oil in the walls of the thus impregnated container. The oil used in these applications does not necessarily have to be all of the type of China-wood oil, because excellent drying results can be obtained on mixtures of China-wood oil with other oils if only care 60 has been taken to have a sufficient proportion of China-wood oil present so that the desired drying effect is obtained by the action of the diacyl peroxide on the elaeostearin present. It is also clear that various combinations and mixtures of 65

diacyl peroxides may be used. If desired a small amount of the ordinary commercial driers can be used in addition to the diacyl peroxides.

No claim is made herein, to any application of the herein described coating compositions to rubber containing sulphur or other vulcanizing agents, vulcanization accelerators or normal reaction products thereof.

The expression "non-reactive material" is intended to exclude rubber, vulcanized rubber, vulcanization accelerators, vulcanizing agents and the reaction products of such materials, which substance are well known to be "reactive" to and injurious to the ordinary heavy metal driers which have heretofore been extensively used in coating compositions containing drying oils, and which interfere with the drying of such coating compositions.

By the term "paint" I mean a composition which is of such a fluid consistency that it can be applied to surfaces by means of a brush dipped into the said paint. The ratio of liquid vehicle to pigment is high, so that the entire paint would be considered as a liquid mass. By the term "printing ink" I mean compositions having the composition of a relatively stiff paste. In speaking of "quick drying paint", I mean that the paint will dry on a glass surface, in substantially less than 48 hours, and in speaking of "quick drying" printing ink, I mean that the printed sheet can be overlaid with another printed sheet, within some seconds, or at any event a few minutes after the printing operation, without smutting, and without the need of using smut sheets. "Varnishes" are analogous to "paints", in that they can be applied as a liquid.

What I claim is:

1. A quick drying coating composition for application to a non-reactive material, which composition contains as a part at least of the vehicle, a bodied drying oil of the type consisting largely of elaeostearin, said composition contain-

ing a major fraction of one percent by weight of dibenzoyl peroxide, based on said drying oil, functioning as the essential oxidation and polymerization catalyst, for the elaeostearin.

2. A quick drying coating composition for application to a non-reactive material, which composition contains a bodied drying oil of the type consisting largely of elaeostearin, said composition being substantially free from heavy metal drier compounds, and containing active oxygen in amount equal to about 0.01% to 0.25% by weight of the said oil, said active oxygen being in the form of a diacyl peroxide, said peroxide functioning as the essential oxidation and polymerization catalyst.

3. A quick drying bodied China-wood oil composition containing a diacyl peroxide dissolved in bodied China-wood oil, said peroxide providing about 0.01 to 0.25% of active oxygen, based on the amount of said oil, which composition will dry in about four hours.

4. A quick drying varnish containing a bodied drying oil consisting largely of elaeostearin as the essential drying oil, and containing not substantially over 0.25% active oxygen based on the said drying oil content, in the form of a diacyl peroxide as the essential oxidation and polymerization catalyst, and which varnish will dry hard in not substantially over seven hours.

5. A quick drying brushable paint which contains a bodied drying oil of the type consisting largely of elaeostearin as the essential drying oil, and a diacyl peroxide as the essential oxidation and polymerization catalyst, the amount of said peroxide corresponding to about 0.01% to 0.25% of active oxygen, based on the amount of said oil, and which paint, when spread upon a board will dry in the air, in not substantially over 5 hours.

FRANCISCUS VISSERT HOOFT.